

## UNITED STATES PATENT OFFICE

2,319,250

## HEAT TREATED COPPER-NICKEL-MOLYBDENUM STEEL ARTICLE AND PROCESS OF MAKING THE SAME

John Mitchell, Chicago, Ill.

No Drawing. Application July 17, 1941,  
Serial No. 402,850

7 Claims. (Cl. 148—21.5)

In accordance with the present invention, there is provided an improved ferrous alloy or steel which possesses high strength coupled with high ductility and corrosion resistance under stress.

One object of the present invention is to produce a steel which possesses improved properties that render it especially suitable for use as chain steel and for the production of the so called "sucker rods" employed in oil well drilling operations, as well as other applications requiring improved fatigue and corrosion resisting properties together with higher ultimate strength without loss of ductility.

Further objects and advantages of the present invention will become apparent as the description proceeds and the features of novelty will be pointed out in detail in the appended claims.

In its specific aspects, the present invention pertains to a copper-nickel-molybdenum steel; and while sucker rods may be regarded as a specific adaptation of the invention, it will be apparent that it is adapted for many uses which require high strength combined with high ductility and resistance to corrosion under stress.

Taking sucker rods as a specific example, it may be noted that ordinarily corrosion-fatigue-resistant sucker rods are made from steels of approximately 0.20% carbon, 0.70% manganese, 1.75% nickel, 0.20%—0.30% molybdenum, the alloy being normalized to produce 85,000—90,000 psi ultimate strength with high ductility or normalized and drawn to produce approximately 80,000—85,000 psi ultimate strength with high ductility. These sucker rods are produced also from steels called low metalloid steels or irons containing low carbon (approximately 0.07%), manganese 0.20% maximum, nickel 3.50%, molybdenum 0.25%, quenched and tempered to approximately 65,000 psi with accompanying high ductility. Both of these steels function well in corrosive media under stress, the former permitting the smallest possible rod size due to its strength with fair corrosion resistant results. The latter alloy is superior in corrosion resistance, but is not always feasible or economical to use in pumping of deep wells due to the low strength which necessitates increased rod size.

The steel of the present invention constitutes a definite improvement over the foregoing al-

loys. It is adapted particularly to applications where the maximum corrosion resistance is required when the parts are subject to tensile stresses, compressive stresses, torsional stresses, bending stresses, and/or alternations of each, in the presence of corrosive media existing individually as salt or saline waters, sulphuric or hydrochloric acids or existing as combinations of such mineral acids and/or in the presence of hydrogen sulphide gas, and/or crude petroleum oils, and the present alloy possesses highly improved corrosion fatigue, together with the requisite high strength and ductility.

The alloy of the present invention contains carbon from about 0.03% to about 0.40%; manganese 0.21% to about 4.00%; phosphorus from the usual amounts present in all steels, i. e., from about 0.005% to about 0.20%; silicon up to about 0.50%; nickel from about 0.50% to about 5.00%; copper from about 0.50% to about 2.00%; and molybdenum up to 0.5%, the balance being substantially all iron.

A typical analysis and physical properties of the present improved steel are as follows:

Carbon 0.08%; manganese 0.32%; silicon 0.24%; phosphorus 0.040%; sulphur 0.015%; nickel 3.22%; copper 1.15%; molybdenum 0.28%, balance substantially iron.

This composition has the following as-rolled properties:

|                                 |        |
|---------------------------------|--------|
| Yield point, psi                | 70,000 |
| Ultimate strength, psi          | 93,000 |
| Elongation in 2 inches per cent | 38     |
| Elongation in 4 inches do       | 25     |
| Elongation in 8 inches do       | 19     |
| Reduction of area do            | 65     |
| Charpy impacts ft. lbs          | 55     |
| Izod impacts do                 | 100    |

40 The tensile tests were pulled in full section  $\frac{3}{4}$ " round.

The desired physical properties of the improved alloy are obtained by heating the steel to a temperature in excess of the  $Ac_3$  point, followed by cooling in air to approximately  $700^{\circ}$  F. or less, followed by reheating to approximately  $825^{\circ}$  F. to  $1200^{\circ}$  F., followed by cooling in air. This reheating operation to  $825^{\circ}$  F. to  $1200^{\circ}$  F. ordinarily reduces the strength of the steel so treated whereas in the improved alloy of this invention

the steel or iron actually increases in strength with no appreciable decrease in ductility. Where steels or irons increase in strength in this operation, the term "accelerated age hardening" or "precipitation hardening" applies, either of which is referred to hereinafter as normalizing and drawing, or where the hot-rolled bar is drawn.

Typical properties of the improved composition as normalized from 1650° F. are as follows:

|                        |          |
|------------------------|----------|
| Yield point, psi       | 62,000   |
| Ultimate strength, psi | 86,900   |
| Elongation in 2 inches | per cent |
| Elongation in 4 inches | do       |
| Elongation in 8 inches | do       |
| Reduction of area      | do       |
| Charpy impacts         | ft. lbs  |
| Izod impacts           | do       |

Typical physical properties when normalized at 1650° F. and drawn at 1000° F., or as-rolled, air-cooled and drawn at 1000° F. are as follows:

|                        |          |
|------------------------|----------|
| Yield point, psi       | 70,000   |
| Ultimate strength, psi | 94,000   |
| Elongation in 2 inches | per cent |
| Elongation in 4 inches | do       |
| Elongation in 8 inches | do       |
| Reduction of area      | do       |
| Charpy impacts         | ft. lbs  |
| Izod impacts           | do       |

All the above tensile properties were determined on the full section of  $\frac{3}{4}$ " round bar. The Izod tests were machined to standard dimensions after treatment.

In the foregoing, the term "normalized" refers to heating above the  $Ac_3$  point and cooling in air; the term "normalized and drawing" referring to heating above the  $Ac_3$  point, cooling in air followed by reheating to any temperature below the  $Ac_1$  point, followed by cooling in air; the term "quenching and tempering" as used herein referring to heating to a temperature in excess of the  $Ac_3$  point, followed by sudden cooling in a liquid medium, followed by reheating to any temperature below the  $Ac_1$  point, followed by cooling in air.

In accordance with the present invention, the desired physical properties are obtained by heating the improved alloy to a temperature in excess of the  $Ac_3$  point, followed by cooling in air to approximately 700° F. or less, followed by reheating to approximately 825° F. to approximately 1200° F., followed by cooling in air. While in the case of the steels of this type of the prior art, this reheating to 825° F.-1200° F. ordinarily reduces the strength of the steel so treated, in the case of the steels of the present invention the reheating actually increases their strength with no appreciable decrease in ductility.

The proper balance of the alloying elements of the present invention when normalized and drawn, produces in sizes up to about one inch cross section an ultimate strength of about 95,000 psi. This is 30,000 psi in excess of the values obtainable with low metalloid irons and also is in excess of the normalized steels commonly used for the purposes for which the present improved alloy is suitable. As to corrosion fatigue, the actual comparison of the present improved alloy in corrosion fatigue tests subjected to an outer fiber stress of 30,000 psi in the presence of a corrosive medium simulating the composition of natural occurring oil well liquids and hydrogen sulphide gas, with air excluded, has run 2,000,000

cycles of stress to failure as compared with 1,000,000 cycles ordinarily obtained with the said standard alloys.

As has been indicated above herein, the present improved steel is adapted particularly to applications where the maximum corrosion resistance is required when the parts are subject to tension, compression, torsion, bending stresses, and/or alternations of each; in the presence of corrosive media existing individually as salt or saline waters, sulphuric or hydrochloric acids, or existing as combinations of such mineral acids and/or in the presence of hydrogen sulphide gas.

The present improved alloy also is adapted to chain steel or similar applications where the parts come in contact with hot metal, reaching temperatures up to 1000° F. which reduce the strength of quenched and tempered chain steels of commonly used compositions, but which, on the other hand, do not affect the strength of the present improved steel.

It will be seen from the foregoing that the specific heat treatment to obtain the maximum properties of the improved alloy consists in normalizing by heating to any temperature above the  $Ac_3$  point, and cooling in air, this normalizing being followed by reheating to a temperature between about 800° F. to about 1200° F., and cooling in air, or by using the single treatment of drawing, between 800° F. to 1200° F. without any prior treatment, when hot-rolled material is hot-finished above the  $Ac_3$  point.

Thus, for example, in accordance with the present invention there are produced heat treated steel articles having excellent corrosion resistance as indicated above, such articles being composed of carbon approximately 0.1%, manganese approximately 0.4%, copper approximately 1%, nickel approximately 3.5%, and molybdenum approximately 0.2%, the balance being iron except for normally present impurities, the articles being characterized by a normalized structure produced by normalizing the steel from a temperature above its  $Ac_3$  point, then reheated to between approximately 800° F. to approximately 1200° F. and then cooled in air.

As illustrative of such articles, there are produced oil well sucker rods composed of a steel consisting of not more than 0.3% carbon, from approximately 0.5% to approximately 1.25% copper, from approximately 1.5% to approximately 3.5% nickel, and from approximately 0.2% to about 0.5% molybdenum, remainder iron except for normal impurities, the sucker rod being characterized by having a normalized and drawn structure imparted by being normalized from above the  $Ac_3$  point of the steel, reheated to a temperature between 800° F. and 1200° F., cooled again in air, and drawn at a temperature between 800° F. and 1200° F.

I claim:

1. An oil well sucker rod composed of a steel consisting of not more than 0.3% carbon, from approximately 0.5% to approximately 1% of manganese, from approximately 0.5% to approximately 1.25% copper, from approximately 1.5% to about 3.5% nickel, and from approximately 0.2% to about 0.5% molybdenum, remainder iron except for normal impurities, the sucker rod being characterized by having a normalized and drawn structure imparted by being normalized from above the  $Ac_3$  point of the steel, reheated to a temperature between 800° F. and 1200° F., cooled again in air and drawn at a temperature between 800° F. and 1200° F.

2. An oil well sucker rod composed of a steel consisting of 0.1% carbon, 0.4% manganese, 1% copper, 3.5% nickel, and 0.2% molybdenum, with the balance substantially all iron, the sucker rod being characterized by a normalized and drawn structure imparted by normalizing the steel from the  $Ac_3$  point of the steel, reheating to a temperature of from approximately 800° F. to approximately 1200° F., cooled in air, and drawn at a temperature between 800° F. and 1200° F.

3. A heat treated steel article consisting of carbon approximately 0.1%, manganese approximately 0.4%, copper approximately 1%, nickel approximately 3.5%, and molybdenum approximately 0.2%, the balance being iron except for normally present impurities, the said article being characterized by a normalized structure produced by normalizing the steel from a temperature above its  $Ac_3$  point, then reheated to between approximately 800° F. to approximately 1200° F., and then cooled in air.

4. A method of producing a steel article which is highly resistant to corrosion in the presence of salt water, hydrogen sulphide gas, and mineral acids, the said article being composed of a steel consisting of not more than approximately 0.30% carbon, from approximately 0.5% to approximately 1% of manganese, from approximately 0.5% to approximately 1.25% copper, from approximately 1.5% to approximately 3.5% nickel, from approximately 0.2% to approximately 0.5% molybdenum, balance substantially all iron, which method comprises heating the steel in "as-rolled" or "as-forged" condition to temperatures between approximately 800° F. to approximately 1200° F., cooling in air to approximately 700° F., reheating to from approximately 825° F. to approximately 1200° F., and drawing within this temperature range.

5. A method of producing a steel article which 40

is highly resistant to corrosion in the presence of salt water, hydrogen sulphide gas, and mineral acids, the said article being composed of a steel consisting of not more than approximately 0.30% carbon, from approximately 0.5% to approximately 1% of manganese, from approximately 0.5% to approximately 1.25% copper, from approximately 1.5% to approximately 3.5% nickel, from approximately 0.2% to approximately 0.5% molybdenum, balance substantially all iron, which method comprises hot rolling and hot finishing the steel above its  $Ac_3$  point, and drawing the steel at between 800° F. to 1200° F.

6. A heat treated steel article composed of not more than 0.3% carbon, from approximately 0.5% to approximately 1% manganese, from approximately 0.5% to approximately 1.25% copper, from approximately 1.5% to approximately 3.5% nickel and from approximately 0.2% to approximately 0.3% molybdenum, remainder iron except for normal impurities, the article being characterized by having a normalized structure imparted by being normalized from above the  $Ac_3$  point of the steel, reheated to a temperature between 900° F. and 1200° F., and cooled.

7. The method of producing a heat treated steel article composed of not more than 0.3% carbon, from approximately 0.5% to approximately 1% manganese, from approximately 0.5% to approximately 1.25% copper, from approximately 1.5% to approximately 3.5% nickel, and from approximately 0.2% to approximately 0.3% molybdenum, remainder iron except for normal impurities, which method consists in heating the steel in excess of the  $Ac_3$  point, cooling to 700° F. or lower, reheating to between approximately 800° F. to approximately 1200° F. and then cooling.

JOHN MITCHELL.